

1

3,132,024

## UPGRADING OF OXIDIC COLUMBIUM-TANTALUM MATERIALS

Louis R. Matricardi, Tonawanda, N.Y., assignor to Union Carbide Corporation, a corporation of New York  
No Drawing. Filed Oct. 10, 1960, Ser. No. 61,381  
3 Claims. (Cl. 75—84)

This application is a continuation-in-part of U.S. patent application 4,864, filed January 27, 1960, now abandoned.

The present invention pertains to a process for producing columbium alloys from oxidic columbium-tantalum starting materials. More specifically the present invention pertains to a process for producing columbium alloys having a higher columbium-tantalum ratio than the columbium to tantalum ratio in the columbium-tantalum oxidic starting materials.

Industry is demanding an ever-increasing volume of low-priced columbium alloys for use in various fields. Coupled with the demand for an increased volume of low priced columbium alloys is a stipulation for more stringent product quality.

Tantalum is the major, and most persistent, contaminant of columbium metal and columbium alloys and the separation of tantalum from columbium is extremely difficult because of the sharp similarity in their chemical behavior.

Several methods of solving the tantalum contamination problem have been attempted. They consist of: (1) the employment of natural ores with a high columbium-tantalum ratio; (2) the enrichment of common ores with a high grade columbium oxide (a by-product of tantalum metal production).

The above first method is amenable for use on high grade oxidic ores of columbium which are characterized by columbium-tantalum ratios of up to 50-to-1.

The second method required several refining steps and is considerably more expensive in view of the cost of high grade columbium cake and its relative unavailability.

It is an object of the present invention to provide a process whereby the columbium-tantalum ratio in columbium alloys is upgraded over the columbium-tantalum ratio in the oxidic starting materials to greater than 200 to 1.

Other objects will be apparent from the subsequent disclosure and appended claims.

The above objects are achieved by admixing an oxide of columbium and tantalum with an alloying agent, a fluxing agent and at least one reducing agent selected from the group consisting of aluminum and silicon wherein the amount of the selected reducing agent in less than the effective amount of reducing agent stoichiometrically required to reduce all the oxidic columbium and tantalum values to columbium and tantalum metal and charging the admixture into a suitable furnace for reduction.

Though the above mentioned process accomplishes the objects of the present invention a more preferred embodiment of the present invention comprises admixing an oxide source of columbium and tantalum which has been pretreated to remove tin and phosphorus with an alloying agent, a fluxing agent and at least one reducing agent selected from the group consisting of aluminum and silicon wherein the amount of selected reducing agent is substantially less than the effective amount of reducing agent stoichiometrically required to reduce all the oxidic columbium and tantalum values to columbium and tantalum metal and charging the admixture into a suitable furnace to provide heat to the admixture whereby a reduction reaction is conducted.

The most preferred embodiment of the present invention comprises admixing an oxide of columbium and tantalum which has been pretreated to remove tin and phos-

2

phorous and having a columbium to tantalum ratio of greater than 6:1 with an alloying agent, a fluxing agent and at least one reducing agent selected from the group consisting of aluminum and silicon wherein the amount of selected effective reducing agent is from 40 to 90 percent of the stoichiometric amount of reducing agent required to reduce all the oxidic columbium and tantalum in the starting materials to columbium and tantalum metal.

The columbium-tantalum ratio in the oxidic starting material may vary over a wide range without substantially affecting the capacity of the present novel process for upgrading the columbium-to-tantalum ratio during reduction of the oxides to metal. Examples of suitable starting materials include columbite and other columbium ores, columbium-tantalum oxide products resulting from metallurgical beneficiation and concentration processes including flotation and pyrometallurgical processes. The columbium-to-tantalum ratio in the starting mixture is not restrictive to the materials which can be treated in the present process. Some amount of upgrading can be achieved in the final product irrespective of the ratio of columbium-to-tantalum in the starting materials. The preferred starting material contains a columbium-to-tantalum ratio greater than about 6:1. The starting materials containing the higher columbium-tantalum ratios permit upgrading of the columbium-tantalum ratio in the final alloy without excess loss in the total recovery of columbium metal during reduction.

The preferred oxidic columbium-tantalum starting materials also preferably contain only small amounts of tin and phosphorous. These may be removed by beneficiation, either physical and/or pyrometallurgical, prior to use in the present process. Although the presence of tin and phosphorous in the oxidic columbium-tantalum starting materials of the present process is not detrimental to the process of upgrading the columbium-tantalum ratio it may in some instances be desirable to produce a final alloy containing none or only small amounts of these elements.

The alloying agent may be any element or group of elements which would serve to pick up the reduced columbium and tantalum metal. The use of an alloy pickup material introduces another facet of the present invention, namely, the fact that a useful columbium alloy is produced in the process concurrent with the upgrading of the columbium-tantalum ratio. Examples of a suitable alloying agent would be iron added in the form of iron scrap, iron shot, steel scrap, iron oxide, nickel shot, nickel oxide, or other iron-containing or nickel containing materials. The resulting product in these examples would be ferro-columbium or a nickel-columbium alloy both of which find diverse use in industry. Hereinafter the term alloying agent is defined as encompassing scrap, oxides and pure metals which contain a suitable alloying element as delineated above. The oxides are readily reduced during reduction of the columbium values.

The reductants employed in the present process are elemental aluminum and/or elemental silicon. In some instances it may be desired to use an aluminum-silicon alloy as a reductant.

Since the present process employs less than stoichiometric amounts of reducing agents, the amount of residual reductant in the final product is low.

The stoichiometric amount of reductants utilized in the present process is a most critical consideration. It has been found that decreasing stoichiometric amounts of reductants cause a progressive increase in the ratio of columbium-tantalum in the final alloy. This relationship is more fully shown in the following Table III by specific figures.

The amount of reductant utilized in the present process can be noted in several ways. For the purposes of this application the amounts of "reducer supplied" refers to the total amount of reducer charged into the starting mixture. The amount of "effective reducer" refers to that amount of reducer actually utilized in the reduction of the metals in the final alloy. The amount of reducer supplied will always be greater than the amount of effective reducer because of side reactions with contaminants. Indeed, when oxidic alloying elements are employed, a portion of the reducer supplied will be required to reduce the oxidic alloying elements to metal. In explaining the relationship between the ratio of columbium to tantalum in the final product as compared with the amount of reducer employed in the process, it is most meaningful to use the term effective reducer as the term relating to the reductant.

A fluxing agent is employed in the present process to aid in forming and regulating the acidity of the slag. The acidity of the slag in turn determines slag viscosity, melting point, reactivity with the furnace lining and other factors known to contribute to the successful operation of a metal-slag metallurgical process. The acidity of the slag is preferably maintained within the range of from 1.2 to 0.60 weight ratio of CaO plus MgO to  $Al_2O_3$  or within the range of from 1.0 to 2.0 weight ratio of CaO plus MgO to  $SiO_2$ . The amount of fluxing agent added is adjusted accordingly.

An accelerator, such as sodium chlorate ( $NaClO_3$ ) may be used to aid in the support of self-sustained exothermic reactions by producing a substantial amount of additional heat in addition to acting as a fluxing agent.

Since accelerating agents such as  $NaClO_3$  are commonly used in the metallurgical industry as fluxes as well as heat sources, the choice of fluxing agents is governed by well formulated practice and hereinafter the term fluxing agent will be construed to encompass such accelerators.

Table I shows the analysis of the starting Cb-Ta source. The starting mixture as shown in Table II was heated by an electric arc furnace in a magnesia lined crucible to conduct the reduction reaction. After the reaction began the remaining portion of the starting mixture was charged into the magnesia crucible and allowed to react. After the reaction was completed the slag and resulting columbium ferro and nickel alloys were tapped into molds to solidify.

Table I

| Columbite Analysis, Percent                             | Run No.           |                   |                   |                   |
|---------------------------------------------------------|-------------------|-------------------|-------------------|-------------------|
|                                                         | 1                 | 2                 | 3                 | 4                 |
| $Cb_2O_5$                                               | 65.78             | 67.80             | 67.00             | 67.00             |
| $Ta_2O_5$                                               | 5.68              | 5.76              | 5.08              | 5.08              |
| $TiO_2$                                                 | 2.94              | 1.84              | 2.98              | 2.98              |
| $FeO$                                                   | 3.66              | 3.53              | 3.53              | 3.53              |
| $MnO$                                                   | 2.08              | 2.01              | 1.86              | 1.86              |
| $SnO_2$                                                 | 0.08              | 0.05              | 0.07              | 0.07              |
| $SiO_2$                                                 | 1.16              | 1.16              | 0.78              | 0.78              |
| Carbon                                                  | 0.02              | 0.01              | 0.03              | 0.03              |
| $ZrO_2$ (est.)                                          | 0.40              | 0.30              | 0.30              | 0.30              |
| Mixture Components (Pounds):                            |                   |                   |                   |                   |
| Fused Columbite                                         | 300               | 300               | 400               | 500               |
| Alloying Agent:                                         |                   |                   |                   |                   |
| Steel Scrap                                             |                   |                   | 43                |                   |
| Iron Scale                                              | 48                | 47                |                   |                   |
| Armco Iron                                              |                   |                   |                   | 54                |
| Reducing Agent:                                         |                   |                   |                   |                   |
| Grained Aluminum                                        | 100               | 92.5              |                   |                   |
| Aluminum Shot                                           |                   |                   | 70                | 91                |
| Fluxing Agent:                                          |                   |                   |                   |                   |
| Lime                                                    |                   |                   | 72                | 90                |
| Sodium Chlorate                                         | 30                | 15                |                   |                   |
| Percent of stoichiometric reduced supplied Process used | <sup>1</sup> 81.6 | <sup>1</sup> 81.2 | <sup>2</sup> 64.0 | <sup>2</sup> 67.0 |
| Percent effective reducer                               | 81.6              | 77.1              | 69.5              | 55.8              |
| Cb-Ta ratio in ore                                      | 9.89:1            | 9.92:1            | 11.26:1           | 11.26:1           |
| Cb-Ta ratio in product                                  | 16.9:1            | 28.4:1            | 103.0:1           | 148.4:1           |

<sup>1</sup>(Al) Aluminothermic.<sup>2</sup>(Al) Aluminothermic + power.

An analysis of the final product is provided in the following Table II.

Table II

|    | Product Analysis, Percent | Run No. |       |       |       |
|----|---------------------------|---------|-------|-------|-------|
|    |                           | 1       | 2     | 3     | 4     |
| 10 | Columbium                 | 65.80   | 67.12 | 61.50 | 65.00 |
|    | Tantalum                  | 3.90    | 2.37  | 0.60  | 0.44  |
|    | Titanium                  | 0.90    | 0.34  | 0.06  |       |
| 15 | Iron                      | 19.97   | 21.67 | 30.40 | 31.80 |
|    | Manganese                 | 2.65    | 0.65  | 0.11  | 1.68  |
|    | Tin                       | 0.13    | 0.21  | 0.11  | 0.16  |
|    | Silicon                   | 0.86    | 0.66  | 0.33  |       |
|    | Carbon                    | 0.14    | 0.17  | 0.13  | 0.21  |

The following Tables III and IV illustrate the use of nickel as an alloying agent in the present process.

Table III

|    | Mixture Components (Pounds)                | Run No. 5 |   |   |                         |
|----|--------------------------------------------|-----------|---|---|-------------------------|
|    |                                            | 1         | 2 | 3 | 4                       |
| 25 | Fused Columbite                            |           |   |   | 500.                    |
|    | Alloying Agent:                            |           |   |   |                         |
|    | Electrolytic Nickel                        |           |   |   | 95.                     |
|    | Nickel Oxide                               |           |   |   | 39.                     |
| 30 | Reducing Agent:                            |           |   |   |                         |
|    | Aluminum Shot                              |           |   |   | 99.                     |
|    | Fluxing Agent:                             |           |   |   |                         |
|    | Lime                                       |           |   |   | 48.                     |
|    | Percent of stoichiometric reducer supplied |           |   |   | 65 (Al) Aluminothermic. |
|    | Percent effective reducer                  |           |   |   | 49.5.                   |
|    | Cb-Ta ratio in ore                         |           |   |   | 9.70:1.                 |
| 35 | Cb-Ta ratio in product                     |           |   |   | 74.4:1.                 |

Analysis of the final product is provided in the following Table IV.

Table IV

|    | Product analysis, percent | Run No. 1 |   |   |       |
|----|---------------------------|-----------|---|---|-------|
|    |                           | 1         | 2 | 3 | 4     |
| 45 | Columbium                 |           |   |   | 43.91 |
|    | Tantalum                  |           |   |   | 0.59  |
|    | Nickel                    |           |   |   | 46.32 |
| 50 | Iron                      |           |   |   | 6.36  |
|    | Manganese                 |           |   |   | 1.36  |
|    | Tin                       |           |   |   | 0.13  |
|    | Silicon                   |           |   |   | 0.55  |
|    | Carbon                    |           |   |   | 0.027 |
|    | Titanium                  |           |   |   | 0.05  |

The criticality of the present process lies in the selection of the proper amount of reducing agent with reference to the columbium-tantalum analysis of the starting material. It has been found that a decrease in the amount of reducing agent to as low as 54% of the effective stoichiometric amount required to effect the complete reduction of the columbium and tantalum leads to an upgrading of the columbium to tantalum ratio in the final product to values as high as 200 to 1.

It has also been found that the higher the columbium to tantalum ratio in the starting material, the higher the ratio in the final product for a given amount of effective reducing agent.

The relationship between the amount of effective reducer employed in the the present process and the extent of upgrading or increase in the columbium to tantalum ratio in the present process can be readily seen from the following table. The figures in the following Table V were taken from a graph which was plotted from the results of several runs similar to that shown in Table I above.

| Effective Aluminum<br>reducer, percent: | Ratio columbium-tantalum<br>in product |    |
|-----------------------------------------|----------------------------------------|----|
| 100                                     | 10:1                                   |    |
| 90                                      | 13:1                                   | 5  |
| 80                                      | 23:1                                   |    |
| 70                                      | 46:1                                   |    |
| 65                                      | 66:1                                   |    |
| 60                                      | 98:1                                   |    |
| 55                                      | 170:1                                  | 10 |
| 54                                      | 200:1                                  |    |

From the above Table V it appears that the ratio of columbium to tantalum will continue to increase with the use of decreasing amounts of reductant. In actuality, though successively decreasing amounts of reductant below about 55 percent effective reducer may be utilized to attain higher columbium to tantalum ratios, the limit of the amount of reductant would be largely dictated by economics for it is known that the use of below about 55 percent effective reducing agent results in an excess amount of unreduced columbium oxide passing to the slag. This fact is not a restriction on the operability of the present process but is a consideration in the economics of the present process.

What is claimed is:

1. A process for increasing the columbium to tantalum ratio in columbium alloys over the columbium-to-tantalum ratio in oxidic columbium-tantalum starting materials comprising admixing a columbium-tantalum oxidic starting material, sufficient fluxing agents to maintain a slag having at least one of the weight ratios selected from the group consisting of weight ratios from about 1.0 to about 2.0 of CaO plus MgO to SiO<sub>2</sub> and from about 1.2 to about 0.60 of CaO plus MgO to Al<sub>2</sub>O<sub>3</sub>, material selected from the group consisting of iron oxides, iron, nickel oxides and nickel and at least one reducing agent selected from the group consisting of aluminum, silicon and alloys consisting of aluminum and silicon wherein said reducing agent is supplied in an amount ranging from about 40 percent to 90 percent of the effective stoichiometric amount of reducing agent required to reduce all the said columbium and tantalum oxides to columbium and tantalum metal; heating the admixture to a sufficiently high temperature and for a sufficient time to fuse said admixture and to cause reduction of said columbium oxide in the admixture whereby a columbium alloy is produced, said columbium alloy having a substantially greater ratio of columbium to tantalum than said columbium-tantalum oxidic starting material.

2. A process for increasing the columbium-to-tantalum ratio in columbium alloys over the columbium-to-tantalum ratio in oxidic columbium-tantalum starting materials comprising admixing a substantially tin and phosphorous free columbium-tantalum oxidic starting material having a columbium-to-tantalum ratio of less than about 10:1,

material selected from the group consisting of iron oxides, iron, nickel oxides and nickel, sufficient fluxing agents to maintain a slag having at least one of the weight ratios selected from the group consisting of weight ratios from about 1.0 to about 2.0 of CaO plus MgO to SiO<sub>2</sub> and from about 1.2 to about 0.60 of CaO plus MgO to Al<sub>2</sub>O<sub>3</sub> and at least one reducing agent selected from the group consisting of aluminum, silicon and alloys consisting of aluminum, silicon wherein said reducing agent is supplied in an amount ranging from about 40 percent to 90 percent of the effective stoichiometric amount of reducing agent required to reduce all the said columbium and tantalum oxides to columbium and tantalum metal; heating the admixture to a sufficiently high temperature and for a sufficient time to fuse said admixture and to cause reduction of said columbium oxide and continuing said reduction until a substantially tin and phosphorous free columbium alloy is produced, said columbium alloy having a greater ratio of columbium-to-tantalum than said columbium-tantalum oxidic starting material.

3. A process for treating columbium-tantalum oxidic starting materials having a columbium-to-tantalum ratio of greater than about 10:1 to produce columbium alloys having columbium-to-tantalum ratios in excess of about 80:1 comprising admixing a columbium-tantalum oxidic starting material having a columbium-to-tantalum ratio of greater than about 10:1, material selected from the group consisting of iron oxides, iron, nickel oxides and nickel, sufficient fluxing agents to maintain a slag having at least one of the weight ratios selected from the group consisting of weight ratios from about 1.0 to about 2.0 of CaO plus MgO to SiO<sub>2</sub> and from about 1.2 to about 0.60 of CaO plus MgO to Al<sub>2</sub>O<sub>3</sub> and at least one reducing agent selected from the group consisting of aluminum, silicon and alloys consisting of aluminum and silicon wherein, said reducing agent is supplied in an amount ranging from about 40 percent to about 60 percent of the effective stoichiometric amount of reducing agent required to reduce all the said columbium and tantalum oxides to columbium and tantalum metal; heating the admixture to a sufficiently high temperature and for a sufficient time to fuse said admixture and to initiate reduction of said columbium oxide and continuing said reduction until a columbium alloy having a columbium-to-tantalum ratio of greater than 80:1 is produced.

#### References Cited in the file of this patent

#### UNITED STATES PATENTS

|    |           |                |               |
|----|-----------|----------------|---------------|
| 50 | 781,808   | Carpenter      | Feb. 7, 1905  |
|    | 1,373,038 | Weber          | Mar. 29, 1921 |
|    | 1,415,516 | Bridge         | May 9, 1922   |
|    | 2,150,555 | Leemans        | Mar. 14, 1939 |
|    | 2,183,517 | Leemans        | Dec. 12, 1939 |
| 55 | 2,205,386 | Balke et al.   | June 25, 1940 |
|    | 2,937,939 | Wilhelm et al. | Mar. 24, 1960 |